

## UNITED STATES PATENT OFFICE

2,020,021

EXTREME PRESSURE LUBRICATING  
COMPOSITION

Bruce B. Farrington and Robert L. Humphreys,  
Berkeley, Calif., assignors to Standard Oil Com-  
pany of California, San Francisco, Calif., a cor-  
poration of Delaware

No Drawing. Application November 20, 1933,  
Serial No. 698,930

14 Claims. (CL. 87—9)

This invention relates to new and useful lubri-  
cating compositions and to methods of preparing  
the same. In particular, it relates to the prepa-  
ration of lubricating compositions of the type  
known generally as "extreme pressure lubri-  
cants," such, for example, as will satisfy the severe  
requirements demanded in the proper lubri-  
cation of hypoid and the like gears, and bearing  
surfaces, metal cutting tools, and the like, sub-  
10 jected to unusually heavy loads per unit area of  
bearing surface.

In general, the primary requirement of such  
an "extreme pressure lubricant" is that it shall  
possess high lubricating film strength; preferably  
it also has low rates of wear and low coefficients  
of friction, and it is an object of the present  
invention to disclose and provide a novel type of  
lubricating composition which fulfills these re-  
quirements. It is a further object of this inven-  
tion to disclose and provide extreme pressure  
lubricants that do not suffer a loss or deteriora-  
tion of high film strength, low rate of wear or  
20 low coefficients of friction in long continued use  
under severe conditions, and which have no tend-  
ency to cause gumming or fouling of the lubri-  
cated metal parts or surfaces under such long  
continued service.

As now known, one class of compositions de-  
signed for use as "extreme pressure lubricants"  
30 comprises mineral lubricating oils to which have  
been added, preferably in oil-soluble form, suffi-  
cient amounts of various active agents discovered  
to possess the properties of increasing the film  
strength and/or decreasing rate of wear and/or  
35 decreasing coefficients of friction of the mineral  
oil base to which they have been added. Mineral  
oil lubricants containing added metallic soaps,  
notably lead soaps, and/or sulfurized fatty acids  
or fatty oils, such as sulfurized animal or vege-  
table oils, are examples of such compositions.  
40 Certain of the compositions of this type have the  
very serious defect that they tend to cause gum-  
ming of the metal parts; certain of them tend to  
separate into their constituent parts upon long  
continued subjection to severe operating condi-  
45 tions. Another class of compositions, designed  
for such service comprises mineral lubricating  
oils, either alone or in admixture with fatty oils,  
to which has been added sulfur in elemental or  
50 uncombined form. Compositions containing such

uncombined sulfur have the serious defect that  
they cause undue corrosion and wear of the metal  
parts to be lubricated, or the parts adjacent thereto,  
such as bushings, etc., which result not only  
in deterioration of the said metal parts but lead  
5 directly to a short life of the lubricating compo-  
sitions themselves.

We have now discovered that the addition of  
small amounts of thiocarbonates, in admixture  
with hydrocarbon or fatty lubricating oils, pro-  
10 vide lubricating compositions, which satisfy all  
of the primary requirements of extreme pressure  
lubricants and, in addition, are stable in long  
continued use, do not separate into their constit-  
uent parts and do not tend to gum, foul or cor-  
15 rode metal surfaces.

The amounts of thiocarbonates required to be  
added to hydrocarbon or fatty lubricating oils for  
the preparation of the composition of our inven-  
tion vary somewhat, depending upon the severity 20  
of the service for which they are designed and,  
to some extent, upon the character of the hydro-  
carbon or fatty lubricating stock used as a base;  
these amounts are in all cases small, however,  
compared with the amounts of active agents of 25  
the prior types, and in general vary between  
about 1% and about 5% of the oil base, by weight.

The thiocarbonates to be added to mineral or  
fatty lubricating oils may contain one, two or  
30 three sulfur atoms per thiocarbonate group, and  
may thus correspond to any one of the following  
type compounds:



in which R and R' represent any aliphatic or aromatic radicals, which may or may not contain another thiocarbonate group such as is here de- 40  
scribed; the compositions may contain mixtures  
of any two or more compounds of these types.

In exemplifying the compositions of our inven-  
tion, and in order to point out the variety of thiocarbonates which we have found suitable in the 45  
preparation of compositions of this character,  
reference is made to the accompanying tabula-  
tion, in which R and R' of the above type formulae  
are shown as exemplified by ethyl, amyl, phenyl,  
benzyl and stearyl radicals. It will be ap- 50

parent that a wide variety of other aliphatic and aromatic radicals may be used in compounds of the above type, any and all of which, so long as capable of incorporation in a hydrocarbon or fatty oil base, are suitable for the practice of our invention, and will give results comparable to those shown in the specific examples below.

| 10<br>Example                                      | Sulfur<br>content<br>percent | Amount<br>added<br>percent<br>by weight | Sulfur in<br>final oil<br>solution | Timken<br>film<br>strength<br>steel on<br>steel total<br>load in<br>pounds |
|----------------------------------------------------|------------------------------|-----------------------------------------|------------------------------------|----------------------------------------------------------------------------|
| 15<br>I—Ethyl amyl thiocarbon-<br>ate.....         | 33.3                         | 2.0                                     | 0.67%                              | 570                                                                        |
| II—Amylbenzylthiocarbon-<br>ate.....               | 25.2                         | 2.0                                     | 0.50                               | 540                                                                        |
| 20<br>III—Stearyl benzyl dithiocar-<br>bonate..... | 16.3                         | 2.0                                     | 0.32                               | 340                                                                        |
| IV—Dibenzyl tri-<br>thiocarbon-<br>ate.....        | 28.0                         | 2.0                                     | 0.56                               | 490                                                                        |
| 25<br>V—Diphenyl monothiocar-<br>bonate.....       | 14.0                         | 2.0                                     | 0.28                               | 480                                                                        |
| Mineral oil stock.....                             | None.                        |                                         |                                    | 180                                                                        |

In the respective columns in the above tabulation there are set out: 1st, typical thiocarbonates, representative of a great number which may suitably be used in the practice of our invention; 2nd, the amount of combined sulfur in each of the several thiocarbonates, in percentage by weight; 3rd, the amount of each of the thiocarbonates added to a mineral hydrocarbon lubricating oil base stock (kept uniform in amount here only for the purposes of exemplification); 4th, the amount of sulfur in each of the finished extreme pressure lubricants, in percentage by weight; 5th, the film strength of the finished lubricating compositions, as measured on the Timken machine described by O. L. Maag in the National Petroleum News for November 16, 1932, page 53, article entitled "Extreme pressure lubricants", wherein the "O. K. load in pounds", or the "load carrying capacity" of the lubricant, is directly measured. In the above exemplifying tabulation the same mineral oil stock was used throughout.

In the preparation of the compositions of our invention, the desired thiocarbonate or mixture of thiocarbonates, in suitable amounts, is admixed with a hydrocarbon or fatty lubricating oil and the admixture merely agitated mechanically in order to obtain complete and homogeneous solution. We have found in general that the thiocarbonates are easily soluble in hydrocarbon and fatty oil, and that no difficulty is encountered in incorporating them therein.

A particular feature of our invention lies in the preparation of bases or concentrates containing relatively large amounts of thiocarbonates in admixture with hydrocarbon or fatty oils. Such concentrates may be stored or transported in this form and before actual use in extreme pressure lubrication service may be diluted with the same or other lubricating oil to any desired concentration. Admixtures of the thiocarbonates and lubricating oils containing upward of 50% of our active agents, by weight, may in this way be prepared. In preparing concentrates or bases of this character complete solution of thiocarbonate is not in all cases necessary, although most of them are freely oil-soluble to this extent. Blending agents, such as amyl

or higher alcohols, may be employed as homogenizers in the case of those thiocarbonates not freely oil-soluble to this extent, if desired; incorporation of the less soluble active agents in suspended form, however, is sufficient to allow the thiocarbonates to function in decreasing film strength in actual use.

Obviously the character and viscosity of the lubricating oil to which the thiocarbonate is added will be dependent to some extent upon the character of service to which the composition is ultimately to be put, and we are not to be limited in the character of the lubricating composition used as a base in the preparation of our compositions. For example, we have found that the life of metal cutting tools is very remarkably lengthened by the incorporation of small amounts of thiocarbonates in either the mineral hydrocarbon or fatty oils used ordinarily in this service. Moreover, we have prepared miscible metal cutting oils in which the usual oil component is replaced with an oil containing small amounts of thiocarbonates in solution, and have found that the life of the cutting tools is greatly lengthened and the character of the metal surfaces cut much improved, especially in severe cutting service. Further, semi-solid and solid lubricating greases have been prepared, in the usual manner, wherein small amounts of thiocarbonates have been incorporated in the hydrocarbon and fatty oils ordinarily used therein; the lubricating film strength is in all cases increased to a degree comparable to the increases pointed out in the examples tabulated above.

While we have described in detail the character of our invention and given numerous illustrative examples of the preparation and application of the composition of our invention, we have done so by way of illustration and with the intention that no limitation should be imposed upon the invention thereby. It will be obvious to one skilled in the art that numerous modifications and variations of the above illustrative examples may be effected in the practice of our invention, which, broadly, includes within its scope any and all lubricating compositions containing thiocarbonates incorporated therein.

We claim:

1. A composition of matter comprising an admixture of a lubricating oil and a thiocarbonate.
2. A composition of matter comprising an admixture of a hydrocarbon oil and a thiocarbonate.
3. A composition of matter comprising a hydrocarbon oil containing between about one and about five percent of a thiocarbonate, by weight.
4. A composition of matter containing a hydrocarbon lubricating oil and an organic ester of a thiocarbonic acid.
5. A composition of matter containing a hydrocarbon lubricating oil and an organic ester of a monothiocarbonic acid.
6. A composition of matter containing a hydrocarbon lubricating oil and an organic ester of dithiocarbonic acid.
7. A composition of matter containing a hydrocarbon lubricating oil and an organic ester of a trithiocarbonic acid.
8. A composition of matter containing a hydrocarbon lubricating oil and a compound of the type—



in which R and R' may represent any aliphatic

- or aromatic radical and in which either or both oxygen atoms may be replaced by a sulphur atom.
9. An extreme pressure lubricant containing between about one and about five percent by weight of an ester of a thiocarbonic acid.
10. An extreme pressure lubricant comprising a mineral oil containing between about one and about five percent by weight of admixed amyl benzyl dithiocarbonate.
11. An extreme pressure lubricant comprising a mineral oil containing between about one and about five percent by weight of admixed diphenyl monothiocarbonate.
12. An extreme pressure lubricant comprising a mineral oil containing between about one and
- about five percent by weight of admixed dibenzyl trithiocarbonate.
13. An extreme pressure lubricant base containing an oil and an organic ester of a thiocarbonic acid, capable of dilution with a lubricating oil to produce an extreme pressure lubricant containing between about one and about five percent by weight of the said ester of the said thiocarbonic acid.
14. An extreme pressure lubricant base containing fifty or more percent by weight of an organic ester of a thiocarbonic acid in admixture with an oil.

BRUCE B. FARRINGTON.  
ROBERT L. HUMPHREYS. 15